

# United States Patent [19]

Nouel

[11] Patent Number: 4,996,131

[45] Date of Patent: \* Feb. 26, 1991

[54] **OFFSET PLATE WITH THIN CHROMIUM LAYER AND METHOD OF MAKING**

[76] Inventor: **Jean-Marie Nouel**, 67 rue Miromesnil, 75008 Paris, France, 75008

[\*] Notice: The portion of the term of this patent subsequent to Aug. 15, 2006 has been disclaimed.

[21] Appl. No.: 356,379

[22] Filed: May 23, 1989

**Related U.S. Application Data**

[63] Continuation of Ser. No. 245,658, Sep. 15, 1988, Pat. No. 4,857,436, which is a continuation of Ser. No. 138,289, Dec. 28, 1987, abandoned, which is a continuation of Ser. No. 481,766, Apr. 4, 1983, abandoned, which is a continuation of Ser. No. 168,003, Jul. 14, 1980, abandoned.

[51] Int. Cl.<sup>5</sup> ..... G03C 1/77

[52] U.S. Cl. ..... 430/276; 430/302; 101/458

[58] Field of Search ..... 430/275, 276; 101/458, 101/463.1; 204/51, 6

[56] **References Cited**

**U.S. PATENT DOCUMENTS**

- 748,004 12/1903 Pancost .  
1,215,494 2/1917 Cornwall .  
1,975,239 10/1934 Ungelenk .  
2,004,824 6/1935 MacLean .  
2,584,317 2/1952 Aller .  
2,678,299 5/1954 Geese et al. .  
2,907,273 10/1959 Geese .  
3,161,508 12/1964 Hepner .  
3,188,186 6/1965 Durham .  
3,280,736 10/1966 Schafler et al. .  
3,289,578 12/1966 Grasso .  
3,461,048 8/1969 Mahlstedt .  
3,660,252 5/1972 Giori .  
3,979,212 9/1976 Peters .  
4,115,127 9/1978 Ikeda .  
4,287,288 9/1981 Pigeon .  
4,301,229 11/1981 Sakaki .  
4,410,620 10/1983 Novel ..... 101/458 X  
4,857,436 8/1989 Novel ..... 101/458 X

**FOREIGN PATENT DOCUMENTS**

- 98776 1/1984 European Pat. Off. ..... 101/458  
475902 11/1937 United Kingdom .  
925961 5/1963 United Kingdom .  
936913 9/1963 United Kingdom .  
1172517 12/1969 United Kingdom .  
1187785 4/1970 United Kingdom .

**OTHER PUBLICATIONS**

IBM Tech. Disc. Bulletin, vol. 26, No. 1, Jun. 1983, Junginger; p. 274.

Primary Examiner—Clifford D. Crowder  
Attorney, Agent, or Firm—DeLio & Associates

[57]

**ABSTRACT**

An offset printing plate and method of manufacturing comprising providing a hard, hydrophilic supporting base material of steel, depositing a layer of dull, porous, ink-rejecting chromium directly onto the surface of the steel base material, the chromium layer having a thickness no greater than one micron and being sufficiently thin and porous to permit the desirable properties of hardness and hydrophilicity of the subjacent steel base material to manifest themselves through the chromium layer during printing, and sufficiently thin to permit removal of the chromium layer from a selected area of the offset printing plate by scraping to expose the subjacent surface of the steel base material. A layer of photo-sensitive resist material is then applied to the plate, the photosensitive resist material being hydrophobic and ink-receptive after insulation and being of sufficient thickness to substantially prevent oxidation of the steel base material through the porous chromium layer during the normal storage period of the offset printing plate prior to use. The chromium may be deposited by immersing the hydrophilic steel base material in the chromium plating solution held at a temperature of between 25° and 35° C. for an initial period of time without a plating current, then applying the plating current, followed by cutting the current to produce the dull and porous chromium layer. Alternatively, the chromium deposit may be formed by plating the base material at a temperature of 5° and 8° C.

16 Claims, No Drawings

## OFFSET PLATE WITH THIN CHROMIUM LAYER AND METHOD OF MAKING

This is a continuation of co-pending application Ser. No. 245,658 filed Sept. 15, 1988, now U.S. Pat. No. 4,857,436, issued Aug. 15, 1989, which is a continuation of abandoned application Ser. No. 138,289 filed Dec. 28, 1987 which is a continuation of abandoned application Ser. No. 481,766 filed Apr. 4, 1983 which is a continuation of abandoned application Ser. No. 168,003 filed Jul. 14, 1980.

The present invention relates to new offset plates whose hydrophilic surface has been given a "dull finish" by way of a thin chromium layer.

It is known that offset printing processes use plates having a surface of hydrophilic nature. Said surface should advantageously be given a dull finish, as said dull finish advantageously helps the control work at printing time, on the one hand, and the adherence to said surface of a photosensitive layer, on the other hand.

Said dull finish can be obtained by treating the plate support or the surface made from a hydrophilic material with processes whereby the said surface is etched either mechanically, or chemically, or electrochemically.

The use of chromium to produce the hydrophilic surface of an offset plate has also been widely described. The chromium layers used have considerable advantages where hardness, water-acceptance and appearance are concerned. Indeed, said chromium layers can present a dull surface. Two methods are known to produce, electrochemically, a chromium layer with a dull surface, one consisting in using an electrolytic bath at low temperature (between 5° and 8° C. for example) and the other consisting in using an electrolytic bath at a temperature below normal (between 25° and 35° C.) but with an electrical current cut when the deposit is effected. But in all the known cases, the chromium layer (whether with a shiny or a dull surface) which is to play the part of the water-accepting layer in offset plates should have a substantial thickness (definitely over 1 $\mu$  and generally between 1.5 and 2.8 $\mu$ ).

It has already been suggested to deposit onto supports, hydrophilic layers of chromium of less than 1 $\mu$  thickness. But considering the examples furnished, specialists are well aware that the very thin layers proposed cannot act as water-accepting hard layers as they scratch too easily and are often porous, thus exposing a sub-jacent surface the properties of which are unacceptable in offset printing.

It has been found and this is precisely the object of the present invention, that it is possible to dull the shiny surface of a hydrophilic material, which surface is to be used as hydrophilic surface for an offset plate, by depositing thereon a layer of dull and porous chromium less than 1 $\mu$  thick, and preferably less than 0.5 $\mu$  thick.

The invention therefore consists in depositing over a surface showing the hydrophilic properties required in offset printing, a very thin layer of dull chromium the relative porosity and fragility of which will be accepted precisely because the sub-jacent surface is a water-accepting and ink-refusing surface, but which will be used to give a "dull finish" to the surface of the final material.

Hydrophilic surfaces which can be "dulled" according to the invention are all surfaces which, heretofore, have been considered as hydrophilic surfaces suitable for offset plates.

For example, it is possible to "dull" with a fine layer of chromium, shiny or semi-shiny surfaces of hard materials such as stainless steel, nickel-tin, chromium itself, chromium-chromium oxide surfaces (used as a coating on steel in certain types of cans), phosphorus-nickel, tin alloys and nickel alloys.

It is also possible, if necessary, to "dull" the surfaces of softer shiny materials such as tin or zinc; but considering the "soft" nature of these metals (and in particular of tin) it is preferable to dull only the surface of the thin layers of tin (i.e. of less than 1 $\mu$  thickness) deposited on a hard surface.

In order to obtain a dull coating of chromium according to the invention, the already known electrochemical techniques are used, which techniques involve either the use of a cold bath or the use of a current cut during the deposit operation. It has however been found that it was possible to obtain the dull chromium deposit directly when using for the baths a temperature below normal (25°-35° C.) and without any current cut, whenever the chromium coating is applied to a chromium or tin surface.

The following examples are given nonrestrictively to illustrate the invention.

### EXAMPLE 1

A stainless steel plate of 35/100 thickness with a shiny surface is used. Said plate is anode scoured, rinsed and then immersed in a conventional chromium bath (250 g/l of chromic anhydride and 2.5 g of sulfuric acid per liter, temperature: 28°). The plate is connected to the cathode; the current (15<sup>4</sup> dcm<sup>2</sup>) is switched on 15 minutes after the immersion of the plate and it is kept on until the chromium deposit has reached a thickness of 0.3 $\mu$ , the current being cut 15 seconds after the beginning of the chromium depositing operation.

A plate with a dull finish is obtained. Said plate is covered with a commercial photosensitive printing layer (PCAS) of approximately 1.8 $\mu$  thickness. After drying (3 mins. at 45° C. and 5 mins. at 85° C.) the plate is ready.

The plate is thereafter used in the conventional manner in offset printing processes: insulation, removal of soluble parts, sizing, etc. . .

Then the plate is used on an offset printing machine. It is then noted:

that the printing layer adheres solidly to the dull chromium surface,  
that the exposed hydrophilic parts are definitely ink-refusing.

After a printing run of 60,000 sheets, it was noted that the dull chromium had been scratched by a hard object contained in the paper, said scratch exposing the stainless steel but the printing had not been affected by it.

### EXAMPLE 2

An offset quality steel plate produced by the company USINOR is used, of 35/100 thickness.

After scouring, rinsing and an etching rinse, a layer of 0.6 $\mu$  thick of hard and shiny chromium is applied on both sides of the plate in a bath composed of:

250 gr/l of chromic anhydride  
2 g/l of sulfuric acid  
Temperature: 45° C.  
Density: 15<sup>4</sup> dcm<sup>2</sup>.

The plate is thus coated on both its faces with a smooth, hard and shiny layer of chromium which will protect adequately the plate during manipulations.

Said plate is then immersed in an electrolytic bath of chromium of similar composition to that described above, but the operational temperature is 28° C. and a layer of 0.4 $\mu$  thickness of chromium is deposited, under 30<sup>4</sup> per dcm<sup>2</sup>, on only one of the faces of the plate.

There is thus obtained a plate which is protected over all its faces by a smooth layer of chromium, and which is coated on one face with a layer of dull chromium for use in offset printing. Then a photosensitive printing layer is deposited on the dull surface and a ready-to-use offset plate is obtained.

### EXAMPLE 3

A chromium plated plate sold by the company SOL-LAC is used as starting plate.

After hot scouring (65° C.) in a sodium bicarbonate bath (100 g/l), the plate being made a cathode, said plate is introduced in a chromium bath with a view to depositing on one of its faces, a thin layer (0.3 $\mu$  for example) of dull chromium.

Similar tests have been conducted using as starting material:

a steel plate (35/100 thick) produced by the company USINOR, on which has been applied beforehand a layer of 0.9 $\mu$  of tin-nickel alloy,

a plate of galvanized steel (thickness 35/100, reference El, sold by the Société de Fer Blanc), with 2.8 g of tin per m<sup>2</sup> over each one of its faces,

a steel plate of 35/100 whose surface has been sanded; it is possible on such a plate to apply the dull chromium coating according to the invention (of less than 1 $\mu$  thickness) without using a current cut during the electrolysis,

a steel plate (35/100 thickness) produced by the company USINOR on both sides of which has been coated a chromium, 0.6 $\mu$  thick of the micro-cracked type supplied by Etablissements WALBERG, reference W.S.A. 2300 and working at 42°. This type of chromium is very resistant to corrosion,

a steel plate (35/100 thickness) produced by the company USINOR on both sides of which has been applied a crack-free chromium layer of 0.6 $\mu$  thickness supplied by Etablissements WALBERG, reference W.S.A. 2650 and working at 65°. This type of chromium is very resistant to corrosion.

All the plates prepared this way have proved to be very good offset plates, capable, without any baking of the photohardened layer, of reaching an output of over 40,000 impressions.

What is claimed is:

1. A method of manufacturing an offset printing plate, comprising:

providing a hard, hydrophilic supporting base material of steel;

depositing a layer of dull, porous, ink-rejecting chromium directly onto the surface of the steel base material, said chromium layer having a thickness no greater than one micron and being sufficiently thin and porous to permit the desirable properties of hardness and hydrophilicity of the subjacent steel base material to manifest themselves through the chromium layer during printing, and sufficiently thin to permit removal of the chromium layer from a selected area of the offset printing plate by scraping to expose the subjacent surface of the steel base material; the step of depositing comprising the steps of:

immersing the hydrophilic steel base material in an electrolytic chromium plating solution for an initial period of time without applying a plating current;

maintaining the temperature of the plating solution at a temperature between 25° and 35° C.; subsequently applying a plating current; and cutting the current to produce the dull and porous chromium deposit having a thickness no greater than one micron; and

applying a layer of photosensitive resist material to the plate, said photosensitive resist material being hydrophobic and ink-receptive after insulation and being of sufficient thickness to substantially prevent oxidation of the steel base material through the porous chromium layer during the normal storage period of the offset printing plate prior to use.

2. A method of manufacturing an offset printing plate according to claim 1 wherein the steel plate is first roughened to form a dull surface.

3. A method of manufacturing an offset printing plate according to claim 2 wherein the roughening of the printing plate is accomplished by anode scouring.

4. A method of manufacturing an offset printing plate according to claim 2 wherein the roughening of the printing plate is accomplished by mechanical abrasion.

5. A method of manufacturing an offset printing plate according to claim 1 wherein the plating current is cut to produce a chromium deposit having a thickness no greater than 0.3 microns.

6. A method of manufacturing an offset printing plate according to claim 1 wherein the steel base material is immersed in the electrolytic chromium plating solution for an initial period of approximately 15 minutes or less without applying a plating current.

7. A method of manufacturing an offset printing plate according to claim 1 wherein the temperature of the plating solution is maintained at a temperature of approximately 28° C.

8. A method of manufacturing an offset printing plate according to claim 1 wherein the plating is accomplished at a current density of approximately 30 amperes per square decimeter (A/dcm<sup>2</sup>) or less.

9. A method of manufacturing an offset printing plate according to claim 8 wherein the plating is accomplished at a current density of approximately 15 amperes per square decimeter (A/dcm<sup>2</sup>).

10. A method of manufacturing an offset printing plate according to claim 1 wherein the plating current is cut after approximately 15 seconds.

11. An offset printing plate manufactured according to claim 1.

12. A method of manufacturing an offset printing plate, comprising:

providing a hard, hydrophilic supporting base material of steel;

depositing a layer of dull, porous, ink-rejecting chromium directly onto the surface of the steel base material, said chromium layer having a thickness no greater than one micron and being sufficiently thin and porous to permit the desirable properties of hardness and hydrophilicity of the subjacent steel base material to manifest themselves through the chromium layer during printing, and sufficiently thin to permit removal of the chromium layer from a selected area of the offset printing plate by scraping to expose the subjacent surface of

the steel base material; the step of depositing comprising the steps of:  
 immersing the hydrophilic steel base material in an electrolytic chromium plating solution;  
 maintaining the temperature of the plating solution 5  
 at a temperature of between 5° and 8° C.; and  
 applying a plating current to produce the chromium deposit having a thickness no greater than 1.0 micron; and  
 applying a layer of photosensitive resist material to 10  
 the plate, said photosensitive resist material being hydrophobic and ink-receptive after insoluation and being of sufficient thickness to substantially prevent oxidation of the steel base material through 15  
 the porous chromium layer during the normal storage period of the offset printing plate prior to use.

13. A method of manufacturing an offset printing plate according to claim 12 wherein the plating current 20  
 is applied until the thickness of the chromium deposit reaches a thickness no greater than 0.5 microns.

14. An offset printing plate manufactured according to claim 12.

15. An offset printing plate comprising: 25

6  
 a supporting base material of steel having a hard hydrophilic surface;  
 a layer of dull, porous, ink-rejecting chromium plated onto the hard surface of the base material, said chromium layer being of thickness no greater than one micron and being sufficiently thin and porous to permit the desirable properties of hardness and hydrophilicity of the subjacent surface to manifest themselves through the chromium layer during printing, and sufficiently thin to permit removal of the chromium layer from a selected area of the offset printing plate by scraping to expose the subjacent hydrophilic surface; and  
 a layer of photosensitive resist material applied directly to the chromium, said photosensitive resist material being hydrophobic and ink-receptive after insoluation and being of sufficient thickness to substantially prevent oxidation of the steel base material through the porous chromium layer during the normal storage period of the offset printing plate prior to use.

16. An offset printing plate according to claim 15 wherein the layer of chromium is less than 0.5 microns thick.

\* \* \* \* \*